

## UNITED STATES PATENT OFFICE

2,388,059

## LUBRICANT

Robert D. Herlocker, Hammond, and Milton Paul Kleinholtz, East Chicago, Ind., and Franklin M. Watkins, Chicago, Ill., assignors to Sinclair Refining Company, New York, N. Y., a corporation of Maine

No Drawing. Application April 24, 1943.  
Serial No. 484,471

5 Claims. (Cl. 252—50)

This invention relates to an improved turbine oil. It relates more particularly to a lubricating oil composition consisting principally of a petroleum lubricating oil, the characteristics of the oil being modified by the addition thereto of a relatively small proportion of a diaminomethane derivative of the class represented by the structural formula:



where  $R_1 N$  is a piperidino radical;  $R_2$  is either hydrogen or an alkyl or an aryl radical,  $R_3$  and  $R_4$  are alkyl or aryl radicals or else  $N R_3 R_4$  is a second nitrogen-containing heterocyclic radical, for instance piperidino. The piperidino radical may be represented by the structural formula:



A lubricating oil composition to be used as a turbine oil, and especially in modern marine steam turbines, is subject to very exacting requirements. Not only must it perform the ordinary function of lubricating the turbine over prolonged periods without interruption but usually it must serve as a coolant, to lubricate the gearing mechanism, to operate oil-actuated governors or control mechanisms having very nice tolerances and lubricate other auxiliary equipment.

Many lubricating oil compositions highly satisfactory for the lubrication of other mechanisms have been found wholly unsuitable for use as a turbine oil. This is probably due primarily to the fact that in normal use turbine oils rapidly become contaminated with water. Whatever the cause, it is generally recognized that the performance of a turbine oil is not predictable from conventional tests applicable to other oil lubricants.

An essential characteristic of a satisfactory turbine oil is its ability to avoid the rusting of the metal parts within the oil system of the turbine and auxiliary apparatus under operating conditions.

The use of many lubricating oil compositions, otherwise satisfactory as turbine oils, has resulted in the rusting of metal parts within the oil system with consequent serious interference with the operation of oil-actuated governors and other parts depending upon close tolerances. The results of such rusting not only interfere with the operation of and tend to clog the deli-

cate clearances of the oil system but the products of the rusting appear to catalyze oxidation of the oil with resultant sludge formation which may further aggravate such conditions. The products of such rusting also appear to act as emulsifying agents.

We have discovered that the previously experienced rusting of metal parts within the oil system in steam turbines may be substantially inhibited by incorporating in the oil a minor proportion of a diaminomethane derivative of the class previously identified herein. Compounds of this class found to be especially effective in inhibiting rusting under conditions usually encountered by turbine oils are those in which each nitrogen atom is included in a piperidino radical. Such compounds found to be especially effective in the preparation of our improved turbine oils of the present invention may be exemplified by the following:

Dipiperidino-methane, which we believe to be represented by the structural formula:



Dipiperidino-ethane, which we believe to be represented by the structural formula:



And phenyl dipiperidino-methane, which we believe to be represented by the structural formula:



where  $R_2$  is a phenyl radical.

It will be understood that the foregoing specific compounds are illustrative of the class and that our invention is not limited to the use of these particular compounds but contemplates the use of other members of the class in the compounding of our improved turbine oils.

Many of the compounds suitable for use in compounding our improved turbine oils are known to the art and may be readily prepared by known methods. In general they can be produced as condensation products of amines and aldehydes.

For example, the dipiperidinomethane, referred to herein and in the appended claims, was prepared as follows: 91.5 grams of 93% piperidine (1 mole) was placed in a 250 c. c. Erlenmeyer

flask. To this there was added portionwise with shaking over a period of 15 minutes 44.1 grams of 34% formalin (0.5 mole formaldehyde). During this addition, considerable heat was evolved and the temperature of the mixture increased to about 170° F. Before the addition of the formalin solution was completed, two phases formed in the flask, a lower aqueous phase and an upper organic phase. The lower phase was separated and on salting out with potassium carbonate yielded 2 c. c. of a red liquid. The upper organic phase was distilled, four cuts being taken. The conditions under which the cuts were taken and the amounts thereof were as follows:

| Cut | Overhead temperature | Pressure,<br>mm. mercury | Amount |
|-----|----------------------|--------------------------|--------|
| 1.  | 177° F.              | 2.6                      | 3      |
| 2.  | 174-175.5° F.        | 2.4-2.0                  | 74.3   |
| 3.  | 176-185° F.          | 2.0-2.8                  | 8      |
| 4.  | Residue.             |                          | 3      |

The second cut was found by analysis, by the Dumas Method, to contain 15% nitrogen as compared with the theoretical nitrogen content of 15.38% for pure dipiperidinomethane. At 20° C. it had a specific gravity of 0.9269 and a refractive index of 1.4886. This second cut was equivalent to 81.6% of the theoretical yield. The average molecular refraction of several batches of the product thus prepared was found to be 56.57 as against a theoretical molecular refraction of 56.48 for pure dipiperidinomethane.

The residue, cut four, was a viscous, dark red liquid.

Seven other preparations were made following the procedure substantially as described excepting a slight variation in the purity of the piperidine employed. The products were found to be substantially uniformly effective in our improved turbine oil.

The dipiperidinoethane referred to herein and in the appended claims was prepared as follows: 179 grams of 95% pure piperidine (2 moles) was placed in a 3-necked flask, equipped with a stirrer, and there was added thereto 30 grams of anhydrous potassium carbonate. To this mixture there was added 48.4 grams (1.1 moles) of acetaldehyde over a period of 2 hours, with stirring, the mixture being kept at a temperature below 55° F. during the addition, by cooling. The reaction mixture was allowed to stand overnight and the aqueous potassium carbonate layer removed. The organic layer was then filtered and topped at a temperature of 155° F., and an absolute pressure of 4.5 millimeters of mercury to remove any water and unreacted volatile materials present. It was a dark colored liquid.

The phenyl dipiperidinomethane referred to herein and in the appended claims was prepared as follows: 134.2 grams of 95% pure piperidine (1.5 moles) was placed in a 500 c. c. Erlenmeyer flask and there was added thereto portionwise, over a period of 10 minutes with shaking, 79.5 grams (0.75 mole) of benzaldehyde. During this addition the temperature of the mixture rose to about 185° F. The solution clouded but, before permitting it to solidify, 300 c. c. of hot ethyl alcohol was added. Upon cooling this mixture there was obtained 153 grams of phenyl dipiperidinomethane as a white solid having a melting point of 176-178° F. From the mother liquor and wash liquors there was obtained 15 additional grams of the product.

In referring to dipiperidinomethane, dipiperidinoethane and phenyl dipiperidinomethane herein and in the appended claims, we refer, respectively, to the above-described products, although, of course, we intend to refer by these terms to the same materials by whatever process they may be made. It is understood that our invention is not predicated upon the identification of the addends as a matter of terminology.

In our co-pending application Serial No. 484,470, filed concurrently herewith, we have described and claimed improved turbine oils in which the rusting characteristics of the lubricating oil constituent are modified by incorporating therewith a small proportion of a diamino-methane derivative of a class of chemical compounds including those described and claimed herein. In said application we have described and claimed specifically turbine oils comprising compounds of the general class in which at least one of the nitrogen atoms is included in a morpholino radical. The present invention is directed to turbine oils in which the addend is a specie of the general class in which at least one of the nitrogen atoms, and advantageously each, is included in a piperidino radical.

The turbine oils to which the present application is specifically directed possess certain advantages over those in which the morpholino compound is incorporated particularly with respect to prolonged effectiveness of the addend under conditions where considerable amounts of water become admixed with and are separated from the turbine oil while in use. This advantage is particularly apparent where relatively smaller proportions of the addend are used.

Though our present invention is independent of any theory as to the reasons for this beneficial result, it appears to be due, in part at least, to differences in solubility of the addends in water. For instance, dimorpholinomethane is readily soluble in water, even at room temperature, while the dipiperidinomethane is soluble in water only to the extent of about 0.45% to 0.50% at 140° F.

The lubricating oil constituent of our improved turbine oil may consist of a petroleum lubricating fraction such as ordinary specified for turbine oils. It may with advantage be a highly refined lubricating oil, for instance an acid-treated petroleum lubricating oil fraction or one which has been subjected to solvent refining such as a phenol-treated fraction from East Texas crude. Solvent refined oils have generally been found more resistant to sludging than the acid-treated oils. For example, lubricating oils such as a phenol-treated East Texas neutral (Sample I), and an acid treated fraction from a Mid-Continent crude, (Sample II), having the following characteristics have been used with advantage:

|                                     | Sample I | Sample II |
|-------------------------------------|----------|-----------|
| Gravity, A. P. I.                   | 26.7     | 23.1      |
| Flash, °F.                          | 405      | 440       |
| Fire, °F.                           | 455      | 515       |
| Viscosity at 100° F., S. U. S.      | 227      | 482.5     |
| Viscosity at 210° F., S. U. S.      | 46.8     | 56.1      |
| Viscosity index (Dean and Davis)    | 79       | 55        |
| Pour, °F.                           | +15      | -10       |
| Neutralization number               | 0.025    | 0.025     |
| Saponification number               | 0.28     | 0.13      |
| Carbon residue (Conradson), percent | 0.05     | 0.036     |
| Ash, percent                        | 0.003    | 0.000     |
| Sulfur, percent                     | 0.3      | 0.47      |
| Navy emulsion tests:                |          |           |
| Distilled water                     | O. K.    | O. K.     |
| 1% salt solution                    | O. K.    | O. K.     |
| 1.0 N caustic solution              | O. K./13 | O. K. /15 |
| Emulsifying constituents with steam | None     | None      |

The Navy emulsion tests appearing in the foregoing tabulation and elsewhere herein were carried out as prescribed under the title "Emulsion test for lubricating oils," prescribed in Federal Standard Stock Catalog, section IV (part 5), Federal Specifications for Lubricants and Liquid Fuels, General Specifications (Methods for Sampling and Testing), VV-L-791a (October 2, 1934), Method 320.12.

By incorporating a minor proportion of a compound of the previously identified class in a suitable lubricating oil constituent, rusting of the metal parts within the oil system of the turbine may be materially inhibited. Depending upon the severity of the rusting conditions encountered in service, including temperature, access of air or other oxidizing gases to the oil, amount of water in contact with the oil, and the like, the proportion of the addend used may with advantage be varied from about 0.01% to about 1% by weight of the oil.

For example, the incorporation of 0.05% of any one of the compounds specifically identified herein has been found to result in a clean test specimen or, at most, only a trace of rusting when the turbine oil composition is subjected to the prescribed test for determining rusting characteristics of turbine oil.

The unique requirements of turbine oils have resulted in the formulation of special test methods for determination of the characteristics of the turbine oil, particularly with respect to rusting and oxidation. The results of rusting tests and oxidation tests herein noted were obtained in accordance with methods prescribed by the American Society of Testing Materials and designated, respectively, "A. S. T. M. Specification D-665-42-T for Turbine Oils" and "Proposed Method for Determining Oxidation Characteristics of Turbine Oils, Section III, Technical Committee C, A. S. T. M. Committee D-2, July 2, 1941."

A further essential characteristic of turbine oils is that they do not form objectionable emulsions under conditions of use. Consequently, in the compounding of such oils, it is necessary to avoid the use of addends which might deleteriously affect the emulsifiability of the oil. A notable advantage of our improved turbine oil is that the emulsifying characteristics of the base oil are not adversely affected by the addends of the present invention.

While the compounds previously identified herein and used in the compounding of our improved turbine oils are not effective, when used alone, in preventing oxidation of the oil under conditions of the prescribed turbine oil oxidation test and, in fact, appear to be pro-oxidants, under such conditions, they are compatible with known anti-oxidants, for example bis-(p-dimethylaminophenyl)-methane which may with advantage be used in conjunction therewith in our improved turbine oils in order to combine high oxidation resistance with the anti-rusting characteristics of our turbine oils.

In the compounding of our improved turbine oil, a small amount of an addend of the above-identified class is admixed with a suitable petroleum lubricating oil in the conventional manner of compounding similar oil compositions. In addition to the lubricating oil constituent and the addend previously identified, various other addition agents having the ability favorably to influence the characteristics of the turbine oil may be incorporated in the improved turbine oil of

our present invention further to improve the properties thereof in various respects. The previously noted bis-(p-dimethylaminophenyl)-methane has been used with special advantage further to improve our turbine oil with respect to its oxidation characteristics.

The following examples of turbine oils, and their characteristics with respect to rusting, will serve as specific illustrations of the application of our invention with respect to various addends of the class herein contemplated. Their characteristics with respect to rusting were determined by the previously referred to prescribed method for testing turbine oils. The results of these rusting tests are reported, as is customarily done, in terms of the amount of rusting of the test specimen, the letters A, B, C, D and E having the following significance:

|     |                                |
|-----|--------------------------------|
| A   | Clear specimen, i. e. no rust. |
| B++ | Only trace of rust.            |
| B+  | Up to 5% of surface rusted.    |
| B   | 5% to 25% of surface rusted.   |
| C   | 25% to 50% of surface rusted.  |
| D   | 50% to 75% of surface rusted.  |
| E   | 75% to 100% of surface rusted. |

The rusting characteristics of our improved turbine oils, having the indicated composition and in which the mineral oil constituent was that previously identified as Sample I, were found to be as follows:

|                            | Addend | Addend concentration | Rusting characteristic |
|----------------------------|--------|----------------------|------------------------|
| None                       |        |                      | E                      |
| Dipiperidinomethane        |        | 0.05                 | B++                    |
| Do                         |        | 0.10                 | A                      |
| Do                         |        | 0.20                 | A                      |
| Do                         |        | 0.50                 | A                      |
| Dipiperidinoethane         |        | 0.02                 | C                      |
| Do                         |        | 0.05                 | A                      |
| Do                         |        | 0.20                 | A                      |
| Phenyl dipiperidinomethane |        | 0.02                 | B                      |
| Do                         |        | 0.05                 | A                      |
| Do                         |        | 0.20                 | A                      |

As appears from the results of these tests, though the use of the oil constituent alone resulted in the rusting of 75% to 100% of the surface of the test specimen, the addition of as small an amount as 0.05% of any one of these addends afforded complete or substantially complete protection against rusting and, in most instances, only a very small amount of rusting resulted where even smaller proportions of the addend were used.

The oxidation induction period of the oil designated Sample I was 150 hours. The inclusion of 0.2% of bis-(p-dimethylaminophenyl)-methane in our improved turbine oil containing 0.1% and 0.3%, respectively, of dipiperidinomethane has resulted in increasing the oxidation induction period of the turbine oil to as high as 825 hours and 850 hours. By this inclusion, the rusting characteristics of our turbine oil were unaffected.

We have found that, by the use of relatively small proportions of bis-(p-dimethylaminophenyl)-methane in conjunction with one of the diaminomethane derivatives previously identified, the anti-rusting life of the turbine oils is actually considerably increased. A turbine oil comprising Sample I was the oil constituent and 0.2% dipiperidinomethane was oxidized for 96 hours under the conditions of the oxidation test previously referred to. When subjected to the A. S. T. M. rusting test, this pre-oxidized oil gave

complete protection against rusting. Another portion of the same oil after oxidation for 120 hours did not give complete protection against rusting. Portions of the same Sample I, containing 0.2% dipiperidinomethane, were oxidized for 72 and 192 hours, respectively, and then subjected to the A. S. T. M. rusting test. These pre-oxidized portions gave complete protection against rusting. While some acids were developed during the test, they seemed to have little effect on either the rusting or the etching of the test specimen.

A further notable characteristic of our improved turbine oil is its ability to withstand contamination by water without material separation of the addend from the oil or substantial deterioration of the addend itself.

As previously noted herein, our improved turbine oil of our present invention has been found to be especially resistant to extraction of the addend from the oil by water. This is illustrated by results of tests in which the prescribed rusting-test method is modified by successively removing the water after the prescribed test and repeating the test on the same oil sample with the addition of fresh water and using a fresh test specimen. Thereafter, the water is again removed and the test repeated until rusting of the test specimen results.

By testing in this manner our turbine oil comprising 0.1% of dipiperidinomethane, rusting was not apparent until the test had been repeated seven times while, with an equal concentration of dimorpholinomethane, a trace of rusting appeared on the third test. Using 0.2% of either of these addends, the rusting inhibition was maintained throughout eight successive tests but, where smaller proportions of the respective addends were used, the characteristic of the piperidino compounds of increased resistance to extraction by water is frequently a distinct advantage.

As we have previously stated herein, depending upon conditions of use, the addend may with advantage be used in proportions ranging from about 0.01% to 1% by weight of the oil. Proportions even in excess of 1% may be used but such larger proportions have not usually been found necessary. Though proportions less than 0.01% may be used, such smaller proportions are usually not sufficiently effective. According-

ly, proportions ranging from about 0.01% to about 1% are generally recommended.

We claim:

1. An improved turbine oil which comprises a petroleum lubricating oil containing a proportion, effective to retard rusting, of a diamino-methane derivative of the class represented by the structural formula



where  $R_1 N$  is a piperidino radical,  $R_2$  is selected from the class consisting of hydrogen, alkyl and aryl radicals and  $NR_3R_4$  is a radical selected from the class consisting of nitrogen-containing heterocyclic radicals and nitrogen-containing radicals wherein  $R_3$  and  $R_4$  are either alkyl or aryl.

2. An improved turbine oil which comprises a petroleum lubricating oil containing from about 0.01% to about 1% of a diaminomethane derivative of the class represented by the structural formula



where  $R_1 N$  is a piperidino radical,  $R_2$  is selected from the class consisting of hydrogen, alkyl and aryl radicals, and  $NR_3R_4$  is a radical selected from the class consisting of nitrogen-containing heterocyclic radicals and nitrogen-containing radicals wherein  $R_3$  and  $R_4$  are either alkyl or aryl.

3. An improved turbine oil which comprises a petroleum lubricating oil containing from about 0.05% to about 1% of dipiperidinomethane.

4. An improved turbine oil which comprises a petroleum lubricating oil containing from about 0.05% to about 1% of 1,1-dipiperidinoethane.

5. An improved turbine oil which comprises a petroleum lubricating oil containing from about 0.05% to about 1% of phenyl dipiperidinomethane.

ROBERT D. HERLOCKER,  
MILTON PAUL KLEINHOLZ,  
FRANKLIN M. WATKINS.